

[54] CONTINUOUS CASTING APPARATUS WITH  
TEMPERATURE CONTROL INCLUDING  
SUCCESSIVE LAYERS OF MATERIAL

[76] Inventor: Roy E. McAlister, 5285 Red Rock  
North, Phoenix, Ariz. 85018

[22] Filed: May 23, 1972

[21] Appl. No.: 256,165

Related U.S. Application Data

[63] Continuation-in-part of Ser. No. 868,756, Oct. 23,  
1969, abandoned.

[52] U.S. Cl. .... 164/283, 164/89

[51] Int. Cl. .... B22d 11/12

[58] Field of Search..... 164/81, 82, 89, 273 R,  
164/283; 425/67

[56] References Cited

UNITED STATES PATENTS

|           |         |               |           |
|-----------|---------|---------------|-----------|
| 2,131,307 | 9/1938  | Behrendt..... | 164/273 R |
| 2,363,695 | 11/1944 | Ruppik .....  | 164/81    |
| 3,430,680 | 3/1969  | Leghorn.....  | 164/81    |

Primary Examiner—R. Spencer Annear  
Attorney—John W. Malley, Raymond F. Lippitt et al.

[57] ABSTRACT

A method and apparatus for continually casting molten metal in solid lengths such as rods, tubes, etc. whereby liquid molten metal such as copper is forced from a reservoir through a nozzle having a cross-sectional area which decreases, as the molten metal flows through the nozzle and solidifies, to account for the volumetric change resulting from the liquid to solid phase transformation of the metal. The nozzle is surrounded by layers of fused compounds which have successively lower melting points to optimize heat flow. The position and profile of the liquid solid interface within the nozzle can be altered as described below by controlling the temperature of the liquid metal entering the nozzle as well as the temperature in the nozzle and controlling the pressure of the liquid metal continuously entering the nozzle.

13 Claims, 4 Drawing Figures



PATENTED SEP 4 1978

3,756,306

SHEET 1 OF 2



INVENTOR  
ROY E. MCALISTER

BY  
Cushman, Harley & Cushman  
ATTORNEYS

PATENTED SEP 4 1973

3,756,306

SHEET 2 OF 2



FIG. 3



FIG. 4

INVENTOR  
Roy E. McALISTER

BY  
Cushman, Darby & Cushman  
ATTORNEYS

**CONTINUOUS CASTING APPARATUS WITH  
TEMPERATURE CONTROL INCLUDING  
SUCCESSIVE LAYERS OF MATERIAL**

This application is a continuation-in-part of Ser. No. 868,756 filed Oct. 23, 1969 (now abandoned).

**BRIEF DESCRIPTION OF THE PRIOR ART AND  
SUMMARY OF THE INVENTION**

The invention relates to an apparatus and method for continuously casting solid lengths of metal.

Casting is the process of producing metal shapes by pouring molten metal into molds of the required form where it is allowed to solidify, and has demonstrated over many centuries a number of distinct advantages over other metal forming methods including the ability to form extremely complex objects of virtually unlimited size and having a variety of isotropic properties not possible with other techniques such as cold working or extrusion.

One of the major disadvantages of casting metal in a stationary mold, however, is that a cumbersome number of time-consuming and frequently difficult steps must be carried out before a finished product is produced, including adding the metal to the mold, cooling the metal in the mold under whatever conditions are necessary to achieve satisfactory solidification and then removing the object from the mold after it has solidified and cooled. Even if the mold can be reused, its output of finished objects in a given time is extremely low compared to other metal working techniques such as cold or hot extrusion. One technique which has been used in the past to increase this output and to combine the advantages of casting with the advantages of fast processes such as extrusion in forming solid lengths of rods, pipes, etc., is termed continuous casting and in this technique molten metal is continually forced through an aperture or tunnel which is formed in a suitable solid structure such as a die. The molten metal is also cooled as it is forced through the aperture or tunnel so that a solid length of metal is continually formed and emerges from the aperture or tunnel. This continuous casting technique requires much less production supervision to produce a given amount of final product than conventional casting techniques using conventional molds, and moreover can form lengths at a rapid rate. Even further, in comparison with extrusion processes, the total energy consumption for the final product, which may be a rod, tubing, wire, bar, pipe or other asymmetrical and symmetrical shape, is considerably less, since no energy is necessary to reheat the molten metal after it has solidified for extrusion, nor is any energy expended in cold working or otherwise fabricating and heat treating the solid metal.

However, continuous casting processes have not been totally successful in the past, in part because of the large capital investment required to set up a continuous casting operation and also because the characteristics of the final product have not been satisfactory in several ways. Other methods of casting which are more expensive have been able to produce more satisfactory products. A number of different approaches to improving continuous casting techniques and devices have been tried in the past and the U.S. Pat. to Conlon et al., No. 3,284,859, discloses one such approach. The patents to Hornak et al., 3,125,440, Ruppick, 2,363,695

and Eldred, 2,242,350 disclose other continuous casting devices.

The present invention relates to a continuous casting arrangement and method whereby molten metal is forced through and solidified in a nozzle having a cross-sectional area which decreases as the metal travels through the nozzle, forms a solid length which emerges from the nozzle and is then cut and stored in the usual manner. More particularly, the nozzle, according to the invention of this application is surrounded by layers of fused compounds each layer successively encountered by the metal having a lower melting point so that heat flow is generally from the nozzle to the uppermost layer. Moreover, a number of arrangements and methods are disclosed for controlling the pressure and temperature of the molten metal entering the nozzle and in the nozzle to adjust the location of the liquid-solid interface in the nozzle, thus allowing control of the characteristics of the final product and enabling a number of variables bearing on those characteristics to be adjusted for optimum operation.

Other objects and purposes of the invention will become clear from reading the following detailed description of the drawings.

**BRIEF DESCRIPTION OF THE DRAWINGS**

FIG. 1 shows a continuous casting apparatus for casting a solid rod;

FIG. 2 shows a cross-sectional view of the nozzle of the apparatus of FIG. 1,

FIG. 3 shows a modification of the arrangement of FIG. 1 whereby the pressure and temperature of the liquid metal entering the nozzle can be controlled, and

FIG. 4 shows a detailed view of the novel arrangement of FIG. 3 whereby the temperature is controlled by a succession of layers of fused compounds.

**DETAILED DESCRIPTION OF THE DRAWINGS**

Reference is now made to FIGS. 1 and 2 which show respectively an arrangement for continuously casting a solid length of rod and a cross-sectional view of the nozzle through which the molten metal passes and in which it solidifies. As shown, the liquid metal flows from a large container 20, which serves as a reservoir and which may be made of any material suitable for holding the liquid metal being cast, to the nozzle 22 in the solidifying structure 24, which serves as a mold, via a line 26, which like container 20 may be made of any material suitable for carrying the liquid metal being cast. The molten metal enters the nozzle 22 in an essentially liquid phase and cools as it passes through nozzle 22 to a solid phase so that a solid length 25 of metal in a rod or other configuration emerges from the top of structure 24 to be wound upon a suitable reel and then cut in conventional fashion.

As can be clearly seen in FIG. 2, the cross-sectional area of the nozzle 22 is greatest where the molten metal is received from the line 26 and decreases non-linearly as the liquid metal cools and is forced upward through the structure 24 to emerge as the rod 25. Since the metal enters nozzle 22 as a liquid and exits as a solid, a solid-liquid interface will necessarily exist within the nozzle 22 between a solid and liquid phase and, as discussed in greater detail below, the exact location of this interface, at least in part, determines the properties of the final output product.

It is well known that, as liquid metal cools, it tends to contract and this contraction has for centuries been one of the major problems of casting in a conventional stationary mold. Moreover, it is believed that failure to account for this contraction in previous continuous casting techniques has been the source of many of the problems which have prevented widespread acceptance of the technique. The present invention accounts for this contraction by tapering the cross-sectional area of nozzle 22, as shown in FIG. 2, so as to compensate for the volumetric changes which result from the liquid to solid transformation and so that the liquid metal moving through nozzle 22 contracts at substantially the same rate that the cross-sectional area of nozzle 22 is decreased. This taper in nozzle 22 permits a controlled degree of extrusion of the solid phase from nozzle 22 which improves density, grain orientation and the mechanical and electrical properties of the solid length 25 forming the rod or other shape. Of course, since different metals which can be cast have different rates of contraction, it may be desirable to tailor the nozzle shape and cross section to the type of metal being cast, so that each metal has a nozzle designed specifically for it. Since the arrangement shown in FIG. 1 is designed to operate continuously, only one product, for example copper rod, would ordinarily be produced.

It may be desirable to adjust the location of the solid-liquid interface in the nozzle, for example, to make sure that the rate of change of the cross-sectional area of the nozzle conforms closely to the actual volumetric changes in the liquid to solid transformation or provide changes in certain properties of the output product and this adjustment may be made in one or more of a number of ways. First, the pressure applied to the liquid metal to force it into and through the nozzle 22 and accordingly, the pressure within the nozzle 22 may be controlled to adjust the rate of flow of the liquid through the nozzle and hence the cooling rate and the position of the liquid-solid interface. Secondly, the temperature of the liquid metal entering the nozzle as well as the rate at which the temperature drops as the liquid moves through the nozzle 22 and is solidified can also be controlled in a variety of ways to shift the liquid solid interface as desired.

The pressure exerted upon the liquid metal entering nozzle 22 can be adjusted in several ways. First, the effective head of the liquid metal above the nozzle 22 can be controlled. It may be possible to move the liquid reservoir container 20 vertically or to alter the amount of liquid metal stored therein. Further, as shown in FIG. 1, gas can be pumped into the space above the liquid in container 20 from a source 28 and kept at a variable pressure above atmospheric pressure by source 28 to exert pressure downward upon the metal in the container 20 which is transmitted to the nozzle. Even further, a suitable pressure exerting device 30, shown in FIG. 1, can be used to provide additional control of pressure which is exerted directly upon the liquid metal flowing in the line 26 toward nozzle 22 and that pressure may range from a vacuum to a pressure greater than both the atmospheric pressure and the pressure exerted by the gas above the liquid metal in the reservoir container 20.

Reference is now made to FIG. 3 which shows another continuous casting apparatus with a reservoir container 40 similar to the container 20 in FIG. 2. Like container 20, reservoir container 40 may be a holding

pot, smelter, induction furnace, arc furnace or the like. As in the arrangement shown in FIG. 1, the liquid molten metal is conveyed from container 40 to the structure 42 within which it is solidified by a line 44. From line 44 the metal enters a tapering nozzle 46, similar to the nozzle 22 and moves through it while cooling to emerge as a solid length of metal. Also in common with FIG. 1, a solid-liquid interface exists within nozzle 46 and the location of this interface is controlled by a variety of means. An emergency valve 48 mounted in line 44 between container 40 and nozzle 46 is also shown in FIG. 3 and allows the flow of liquid metal to the structure 42 to be cut off for any reason.

As in the embodiment of FIG. 1, it is contemplated that a source of gas will be associated with the container 40 so that gas pressure above the liquid in container 40 can be used to at least partially control the location of the solid-liquid interface in the nozzle 42. Even further, in this arrangement it is contemplated that more pressure can be added or subtracted to the liquid metal flowing in the line 44 by an induction pump 50, which is supplied with energy from a suitable source 51 and which generates, by means of the coils 53 wrapped around the line 44, a magnetic field which is orthogonal to electrical current generated in the fused copper or other metal flowing in line 44 by a suitable electrical or similar device. In the arrangement of FIG. 3, even more pressure can be exerted upon the line 44 by a piston arrangement 54 in which hydraulic pressure is applied to the liquid metal flowing down line 44.

In addition to controlling the location of the liquid-solid interface by applying pressure to the liquid flowing in the line 44, the arrangement of FIG. 3 contemplates that the temperature of the liquid flowing in line 44 as well as the temperature of the liquid in structure 42 can be controlled to place the location of the interface so that the properties of the final product are as desired.

As shown in FIG. 3, the source of electrical energy 51 also forces current to flow through the liquid in the container 40 or line 44. This current flowing in the line 44 is acted upon by the induction pump and also resistively heats both the liquid metal in the container 40 and the metal flowing through the line 44. Moreover, in the arrangement of FIG. 3, it is contemplated that nozzle 46, which as mentioned above, is similar to the nozzle 22, will be kept at essentially a constant temperature by exchanging heat through a medium 49 of solid and liquid material such as a fused salt. Alternately, temperature control at the nozzle 46 may be accomplished by exchanging heat to a split phase medium consisting of gas and liquid phases so that in the gas generated by the heat exchange process is condensed by the heat exchanger at a point removed from the nozzle and added back to the bath, thereby stabilizing the nozzle temperature. A concentric heat exchanger may also be added around the device 42 if desired to assist in heat removal.

Further, the nozzle temperature can simply be controlled and further cooling of the extruded metal accomplished simply by causing the metal to flow through layers of fused compounds such as shown in FIG. 4, which surround nozzle 60, each higher compound being of a lower melting point so that heat flow is generally caused to be from the nozzle to the uppermost layer. Two or more layers are required and three layers

has been found particularly satisfactory. For example, in the arrangement of FIG. 4, the liquid metal enters the nozzle 60 which may be similar to nozzle 22 from the line 62 and flows in turn through a first layer 64 which may be comprised of a first fused salt at the melting point of 1,000° F. through a second layer 66 which may be another fused salt with melting point of 600° F. and finally through a layer 68 which may, for example, be of liquid lead.

The following table sets forth a number of specific combinations of fused compounds with the first layer being that first encountered by the metal, the second layer being that next encountered, etc.:

|                                  | First Layer    | Second Layer                                      | Third Layer                                           | Fourth Layer   |
|----------------------------------|----------------|---------------------------------------------------|-------------------------------------------------------|----------------|
| Particularly useful for steel    | Pb             | Bi                                                | Mixture of UF <sub>4</sub> , PbF and LiF <sub>2</sub> | Graphite Chips |
| Particularly useful for copper   | Pb             | Graphite Pellets                                  |                                                       |                |
|                                  | Pb             | Boron Nitride                                     |                                                       |                |
|                                  | Pb             | Nitrogen Foam Granules                            |                                                       |                |
| Particularly Useful for copper   | B <sub>1</sub> | Graphite Pellets                                  |                                                       |                |
|                                  | B <sub>1</sub> | Boron Nitride                                     |                                                       |                |
|                                  | B <sub>1</sub> | Nitrogen Foam Granules                            |                                                       |                |
| Particularly useful for aluminum | Pb             | Mixture of PbSO <sub>4</sub> and USO <sub>4</sub> | Graphite Pellets                                      |                |
| Particularly useful for aluminum | Pb             | Mixture of PbSO <sub>4</sub> and USO <sub>4</sub> | Boron Nitride Nitrogen Foam Granules                  |                |

Other heavy salt systems which can be combined together in layers include mixtures of:

UF<sub>4</sub>, L<sub>1</sub>F, NaF, and KF  
PbF<sub>2</sub>, L<sub>1</sub>F, NaF and KF  
PbCl<sub>2</sub>, L<sub>1</sub>Cl, NaCl and KCl  
UF<sub>4</sub>, PbCl<sub>2</sub> and ZnF<sub>4</sub>  
L<sub>1</sub>F and NaF

The layers operate to effectively limit the amount of liquid metal passing through them which can be taken into solution.

The temperature of the liquid flowing in the line 44 may also be controlled as discussed above and one suitable way of controlling such temperature is to simply impinge variable intensity gas flames from the source 52 onto the line 44 connecting the container 40 to the nozzle 42. Similarly, such control can be accomplished by disposing resistive elements 54 about the line 44 and controlling the amount of energy supplied to such resistive heaters.

The various control arrangements shown above are capable of producing a product which is not only superior in such characteristics as grain refinement, seamless detail on tubing pipe, and other manufacturing items, but also results in a remarkable efficiency in producing the product at a considerable economy over previous methods of casting. As mentioned above, the arrangement shown in FIGS. 1-4 in comparison with other methods such as extrusion results in considerably less energy consumption for the preparation of a vari-

ety of products. This energy saving comes about because no reheat energy is required for extrusion, no work energy is encountered in cold working, and no handling energy associated with competitive fabrications such as annealing and heat up for heat treating is necessary. Even further, 100 percent inspection is a simple and easy job.

Thus, in comparison with other continuous casting arrangements, the novel arrangement shown in FIGS. 1-4 is more economical to set up and accordingly requires less capital investment to produce the same products. Moreover, any system for producing a given product can be normally converted to produce other products simply by substituting another nozzle and making other minor adjustments. Since no water is required in this arrangement for cooling the casting, it is believed that this arrangement will be safer than other continuous casting operations requiring water.

Another advantage, in comparison with other continuous casting arrangements, is that this system requires no pickling because the final output metal, such as copper rod, can be coated immediately upon exposure to the air.

Accordingly, the advantages of this type of arrangement which not only produces a superior product in comparison with other continuous casting and noncontinuous casting arrangements, but produces that product cheaper, safer and quicker should be apparent; and the scope of the invention is not intended to be limited only by the scope of the appended claims.

What is claimed is:

1. A continuous casting apparatus comprising:  
a source of molten metal,  
nozzle means for receiving said molten metal so that  
said molten metal is transformed from the liquid to  
solid phase within said nozzle, said nozzle having  
an internal cross-sectional area presented to said  
molten metal which decreases to account for volu-  
metric changes of said metal as said molten metal  
travels through said nozzle means and is trans-  
formed from the liquid to the solid phase,  
means for conveying said molten metal from said  
container to said nozzle, and  
means for controlling the temperature of said nozzle  
means including a plurality of layers about said  
nozzle means through which said molten metal  
flows, each successive layer encountered being of  
lower melting point so that heat flow is generally  
caused to be from said nozzle means to the layer  
having the lowest melting point and each having a  
substantial thickness sufficient to cool molten  
metal passing through said nozzle means.

2. An apparatus as in claim 1 wherein said internal  
cross section varies to account for the volumetric  
changes in the liquid to solid phase transformation to  
improve the density grain orientation and resulting  
chemical and electrical properties of the product cast.

3. An apparatus as in claim 2 including means for  
controlling the temperature of said molten liquid.

4. An apparatus as in claim 3 wherein said tempera-  
ture control means includes means for impinging gas  
flames on said means for conveying said molten metal  
from said source to said nozzle means.

5. An apparatus as in claim 3 wherein said tempera-  
ture control means includes resistance heating means  
for heating said conveying means.

6. An apparatus as in claim 3 wherein said temperature control means includes an induction heater.

7. An apparatus as in claim 2 including means for controlling the temperature of said nozzle means.

8. An apparatus as in claim 2 including means to apply pressure to said liquid metal to control the location of the liquid-solid interface in said nozzle means.

9. An apparatus as in claim 8 wherein said pressure control means includes means for applying gas pressure to the liquid in said source.

10. An apparatus as in claim 8 wherein said pressure control means includes means for applying pressure to liquid in said conveying means.

11. Apparatus as in claim 1 wherein said layers are chosen from the group consisting of:

|                                  | First Layer    | Second Layer                                      | Third Layer                                           | Fourth Layer   |
|----------------------------------|----------------|---------------------------------------------------|-------------------------------------------------------|----------------|
| Particularly useful for steel    | Pb             | Bi                                                | Mixture of UF <sub>4</sub> , PbF <sub>2</sub> and LiF | Graphite Chips |
| Particularly useful for copper   | Pb             | Graphite Pellets                                  |                                                       |                |
|                                  | Pb             | Boron Nitride                                     |                                                       |                |
|                                  | Pb             | Nitrogen Foam Granules                            |                                                       |                |
| Particularly useful for copper   | B <sub>1</sub> | Graphite Pellets                                  |                                                       |                |
|                                  | B <sub>1</sub> | Boron Nitride                                     |                                                       |                |
|                                  | B <sub>1</sub> | Nitrogen Foam Granules                            |                                                       |                |
| Particularly useful for aluminum | Pb             | Mixture of PbSO <sub>4</sub> and USO <sub>4</sub> | Boron Nitride Nitrogen Foam Granules                  |                |
| Particularly useful for aluminum | Pb             | Mixture of PbSO <sub>4</sub> and USO <sub>4</sub> | Graphite Pellets                                      |                |

12. A structure for controlling the location of a solid-liquid interface in a nozzle into which liquid metal is continuously entering and from which solid metal in a given shape is being withdrawn comprising a plurality of layers of fused compounds, each higher layer being of lower melting point than the layer below it so that heat flows from said nozzle to the uppermost layer and each having a substantial thickness sufficient to cool molten metal passing through said nozzle means.

13. A structure as in claim 12 wherein said layers are chosen from the group consisting of:

|    | First Layer                      | Second Layer           | Third Layer                                       | Fourth Layer                                          |
|----|----------------------------------|------------------------|---------------------------------------------------|-------------------------------------------------------|
| 15 | Particularly useful for steel    | Pb                     | Bi                                                | Mixture of UF <sub>4</sub> , PbF <sub>2</sub> and LiF |
| 20 | Particularly useful for copper   | Pb                     | Graphite Pellets                                  |                                                       |
|    | Pb                               | Boron Nitride          |                                                   |                                                       |
|    | Pb                               | Nitrogen Foam Granules |                                                   |                                                       |
| 25 | Particularly used for copper     | B <sub>1</sub>         | Graphite Pellets                                  |                                                       |
|    | B <sub>1</sub>                   | Boron Nitride          |                                                   |                                                       |
|    | B <sub>1</sub>                   | Nitrogen Foam Granules |                                                   |                                                       |
| 30 | Particularly useful for aluminum | Pb                     | Mixture of PbSO <sub>4</sub> and USO <sub>4</sub> | Boron Nitride Nitrogen Foam Granules                  |
| 35 | Particularly useful for aluminum | Pb                     | Mixture of PbSO <sub>4</sub> and USO <sub>4</sub> | Graphite Pellets                                      |

\* \* \* \* \*